# EUROPEAN PATENT SPECIFICATION

(11) **EP 0 561 860 B1**
(45) Date of publication and mention of the grant of the patent: **22.11.1995**
(21) Application number: 92900247.5
(22) Date of filing: 10.12.1991
(51) Int. Cl.: G03C 7/392, G03C 7/413

(54) **METHOD OF DEVELOPING SILVER HALIDE COLOUR PHOTOGRAPHIC MATERIALS AND USE OF PYRAZOLIDONES**
VERFAHREN ZUR ENTWICKLUNG FARBPHOTOGRAPHISCHER SILBERHALOGENIDMATERIALIEN UND VERWENDUNG VON PYRAZOLIDONEN
PROCEDE DE DEVELOPPEMENT DE MATERIAUX COULEUR A BASE D'HALOGENURE D'ARGENT ET UTILISATION DE PYRAZOLIDONES

(30) Priority: 13.12.1990 GB 9027062
(43) Date of publication of application: 29.09.1993
(73) Proprietor: KODAK LIMITED, Harrow, Middlesex HA1 4TY (GB); EASTMAN KODAK COMPANY, Rochester, New York 14650-2201 (US)
(72) Inventor: TWIST, Peter Jeffery c/o KODAK LIMITED, Harrow Middlesex HA1 4TY (GB)
(74) Representative: Baron, Paul Alexander Clifford
(86) International application number: EP9102363
(87) International publication number: WO9210789

(56) References cited:
- EP-A- 0 347 849
- GB-A- 963 988
- JP-A-60 162 253
- US-A- 3 902 905
- US-A- 4 155 763
- US-A- 4 266 002
- US-A- 4 465 762
- US-A- 4 483 919
- US-A- 4 845 016
- PATENT ABSTRACTS OF JAPAN vol. 7, no. 256 (P-236)(1401) 15 November 1983 & JP,A,58 139 136

## Description

This invention relates to photographic silver halide processing solutions and particularly to colour developing solutions.

It is well understood that the parameters of colour development, such as time, temperature, component content, pH, etc have to be carefully controlled in order to obtain consistent sensitometric results. This usually means that there has to be close control over, for example, the temperature and replenishment of colour developing agent. The cost of such control is clearly significant in a commercial operation.

US Patent 4 465 762 discloses silver halide colour materials containing a pyrazolidinone of formula (I). The present pyrazolidinones can only be derived by selecting substituents from two separate lists. No specific such compounds are described.

US Patent 4 266 002 describes the use of pyrazolidinones as an electron transfer agent in a dye diffusion transfer element. No chromogenic dye development is described.

US Patent 4 483 919 describes a photographic colour material containing a compound that releases a pyrazolidinone upon development. The release is therefore imagewise.

US Patent 4 155 763 describes colour developing solutions comprising an aromatic amine colour developing agent and a 1-aryl-pyrazolidone having two substituents at the 4-position of the pyrazolidone. The advantages are said to include faster image dye formation and a more stable colour developing solution. The English language abstract of Japanese application 62/178251 describes a colour developing solution comprising a para-phenylenediamine colour developing agent and an auxiliary developing agent including, *inter alia*, 1-phenyl-pyrazolidone. Image formation is described as "highly sensitive" and forming "excellent gradation". It is also said to be "free from the influence of agitation.

The above two references indicate that the use of a second developing agent in colour developing solutions provides higher developing activity as it would in black and white developer solutions wherein, for example, the activity of a hydroquinone developing agent is very much increased by the addition of Metol or 1-phenyl-pyrazolidone.

The present invention provides a method of developing an imagewise exposed silver halide colour material to provide sensitometric results of reduced variability which comprises
carrying out colour development in an aqueous colour developing solution containing a colour developing agent in the presence of one or a combination of the pyrazolidinone silver halide developing agents of the general formula:
wherein
R¹ and R² are each hydrogen or an alkoxy group having 1-4 carbon atoms, and
R³ and R⁴ are each hydrogen or an alkyl group having 1-10 carbon atoms,
with the proviso that either one of R¹ or R² is an alkoxy group or either one of R³ or R⁴ is an alkyl group of 3-7 carbon atoms,
incorporated in said silver halide colour material in an inactive form from which the active form is released in the alkaline developer solution, *characterised in that* the nature of the pyrazolidinone silver halide developing agent(s) is such that in low activity conditions development is accelerated while in high activity conditions development is decelerated thus reducing the variability in the density versus LogE curve (the characteristic curve) caused by changes in development time.

The pyrazolidinone developing agent may also be present in the colour developer solution.

In the present invention (unlike the prior art) not only are the low activity conditions accelerated by the presently used ETA's but also high activity conditions are decelerated thus leading to less variation in sensitometric results under both high and low activity conditions. This is seen graphically as a compression of the spread of the characterisitic curves as shown in, say, Figs 2 and 3 compared to Fig 1.

When it is incorporated in the photographic material it is in a form which is inactive until processing takes place. For example it could be inactivated by a blocking group which is hydrolysed off when the material is immersed in the developing solution (which is usually alkaline).

A number of ETA's have been examined for their effectiveness in lowering sensitometric sensitivity to process variables. The reduction of sensitivity to development time is used as an example. Three broad types of behaviour for different ETA's can be observed and these are as follows:
(1) A reduction of sensitometric spread with control of Dmin increase caused by time and maintenance of aim contrast. See Fig 10 of the accompanying drawings in which the solid lines represent the control and the broken lines the effect of the added ETA. This convention is also used in Figs 11 and 12.
(2) A reduction of sensitometric spread with control of Dmin increase caused by time and an increase of contrast. See Fig 11 of the accompanying drawings.
(3) A modest reduction in sensitometric spread but with little Dmin control, a reduction in contrast and still a considerable variability. See Fig 12 of the accompanying drawings. These results are clearly not acceptable particularly with respect to the increase in Dmin. The use of Type (3) ETA's alone is therefore not part of the present invention.
   Type (1) is the preferred behaviour exhibited by the preferred compounds. Type (2) is another useful and beneficial behaviour and could, in certain cases, be preferred over Type (1) if an increase in contrast or corresponding trade-off was desired. The present invention also includes the use of combinations of ETA's. Combinations of Type (2) and (3), for example, can give an overall behaviour similar to Type (1). Combinations of Type (1) and (3) also give good results in that the spread of the sensitometric curves is particularly well controlled.

A useful group of Type (1) ETA's of formula (I) are those in which at least one of R¹ and/or R² is an alkoxy group of 1-4 carbon atoms, eg -OCH₃, R³ is hydrogen or an alkyl group of 1-4 carbon atoms, eg - CH₃ and R⁴ is hydrogen or a hydroxyalkyl group of 1-4 carbon atoms, eg -CH₂OH.

A useful group of Type (2) ETA's of formula (I) are those in which R¹, R² and R³ are hydrogen and R⁴ is an alkyl group of 3-7 atoms, eg -C₅H₁₁

The preferred black-and-white developers are: 1-(4-methoxyphenyl)-3-pyrazolidone, 1-(3,4-dimethoxyphenyl)-3-pyrazolidone, and 1-phenyl-4-n-pentylpyrazolidone.

The black-and-white developing agent may be present in the developer solution at a concentration up to 5 g/l preferably in the range 0.05 to 0.5 g/l. When incorporated in the photographic material it may be present in one or more layers thereof. Instead of incorporating them per se in the photographic material they are, as indicated above, in the form of a compound that releases them as a function of the pH of the processing solution.

It has been found, in particular, that the presence of the black-and-white developing agent improves variability caused by variations in time and temperature of development, pH, bromide ion concentration and colour developing agent (eg CD4) concentration in the colour developer solution. The reduced risk of sensitometric variations further means that replenishment rates can be reduced thus resulting in less overflow and effluent. The sometimes needed bromide ion removal from the developer solution may also be avoidable.

The present invention is particularly applicable to the processing of colour negative film but is also applicable to other processes, eg colour paper. The material to be processed comprises a support bearing at least one silver halide emulsion layer having a colour coupler associated therewith. The term "associated therewith" here takes its normal meaning in art. The coupler may be incorporated in the emulsion layer or in a layer adjacent thereto. The preferred colour materials comprise three dye image forming units each containing one or more emulsion layers having couplers associated therewith and each sensitised to a different region of the spectrum. A typical colour material would contain such units sensitised to blue, green and red light and capable of forming yellow, magenta and cyan image dyes respectively.

Examples of colour photographic materials and methods of processing them are described in Research Disclosure Item 308119, December 1989 published by Kenneth Mason Publications, Emsworth, Hants, United Kingdom.

The following Examples are included for a better understanding of the invention.

### EXAMPLE 1

A single layer coating of a silver bromoiodide emulsion comprising tabular grains having a mean grain area of 1.05 mµ² containing a colour coupler (A) of the formula:
dissolved in di-tert-butylphthalate (coupler to solvent ratio of 1:0.5) was coated at 1.0 g/m² (as silver) and 0.6 g/m² of coupler.

The following basic colour developing solution was used:

### Colour Developer

Table 1 below gives process details of concentration of 1-(4-methoxyphenyl)-3-pyrazolidone and development time at 37.8°C.

The sensitometric results for these twelve processes are shown as sets of three time series in Figures 1, 2 and 3 each for a different level of ETA. In Figure 1 (control), without any ETA, the effect of time is considerable giving increases in Dmin, speed, Dmax and contrast. In Figure 2 with 0.1 g/l of ETA the sensitometric spread caused by time is very much reduced. In Figure 3 with 0.3 g/l ETA the curves are even closer together. The optimum level of ETA is probably between 0.1 and 0.3 g/l. The essential difference between this result and that expected is that not only do short process times show acceleration (as might be expected) but the long process times show a reduction (which is not expected).

This unexpected compression of sensitometric spread from both high and low activity conditions is also shown with other process variables as is shown below in Examples 2 and 3.

Similar results were found with the couplers (B) and (C) having the formulae:
coated with the same emulsion and processed in the same solution.

### EXAMPLE 2

A set of experiments with sodium bromide levels from 0.45 to 2.15 g/l and ETA levels of 0, 0.1 and 0.3 g/l was carried out on the same coatings as mentioned above. The results are shown in Figures 4, 5 and 6. Again with zero level of ETA there is a considerable sensitometric spread caused by changing bromide ion level and as the ETA level is increased this is reduced as shown in Figures 5 and 6. The optimum level of ETA is probably between 0.1 and 0.3 g/l.

### EXAMPLE 3

A single layer coating of a silver bromoiodide emulsion as described in Example 1 was tested by the procedure of Example 1 was followed except that the time of development was kept constant at 2.5 minutes while varying the CD4 and ETA concentrations as set out in Table 2 below.

The sensitometric results for these fifteen processes are shown as sets of three CD4 level series in Figures 7,8 and 9. In Figure 7 (control) without any ETA the effect of CD4 level is considerable giving increases in Dmin, speed, Dmax and contrast. In Figure 8 with 0.1 g/l of ETA the sensitometric spread is caused by CD4 is very much reduced. In Figure 9 with 0.3 g/l ETA the curves have separated again but are still better than the control especially in similarity of contrast.

Similar results were found with other couplers (B) and (C) coated with the same emulsion and processed in the same solution.

## Claims

1. A method of developing an imagewise exposed silver halide colour material to provide sensitometric results of reduced variability which comprises
carrying out colour development in an aqueous colour developing solution containing a colour developing agent in the presence of one or a combination of the pyrazolidinone silver halide developing agents of the general formula: wherein
R¹ and R² are each hydrogen or an alkoxy group having 1-4 carbon atoms, and
R³ and R⁴ are each hydrogen or an alkyl group having 1-10 carbon atoms,
with the proviso that either one of R¹ or R² is an alkoxy group or either one of R³ or R⁴ is an alkyl group of 3-7 carbon atoms,
incorporated in said silver halide colour material in an inactive form from which the active form is released in the alkaline developing solution,
the nature of the pyrazolidinone silver halide developing agent(s) being such that in low activity conditions development is accelerated while in high activity conditions development is decelerated thus reducing the variability in the density versus LogE curve (the characteristic curve) caused by changes in development time.

2. A method as claimed in claim 1 in which the pyrazolidinone developing agent is also contained in the colour developer solution.

3. A method as claimed in claim 1 or 2 in which at least one of R¹ and/or R² is an alkyoxy group of 1-4 carbon atoms, R³ is hydrogen or an alkyl group of 1-4 carbon atoms, and R⁴ is hydrogen or a hydroxyalkyl group of 1-4 carbon atoms.

4. A method as claimed in claim 1 or 2 in which R¹, R² and R³ are hydrogen and R⁴ is an alkyl group of 3-7 atoms.

5. A method as claimed in any of claims 1-4 in which the pyrazolidinone developing agent is 1-(4-methoxyphenyl)-3-pyrazolidone, 1-(3,4-dimethoxyphenyl)-3-pyrazolidone, or 1-phenyl-4-n-pentylpyrazolidone.

6. A method as claimed in any of claims 2-5 in which the pyrazolidinone developing agent is present in the developer solution at a concentration of from 0.05 to 0.5 g/l.

7. Use of one or more pyrazolidones to reduce the sensitometric variability of processed photographic silver halide colour materials, wherein the pyrazolidinones have the general formula (I): wherein
R¹ and R² are each hydrogen or an alkoxy group having 1-4 carbon atoms, and
R³ and R⁴ are each hydrogen or an alkyl group having 1-10 carbon atoms,
with the proviso that either one of R¹ or R² is an alkoxy group or either one of R³ or R⁴ is an alkyl group of 3-7 carbon atoms,
and wherein the pyrazolidinone(s) is present during colour development carried out in an aqueous colour developing solution and is such that in low activity conditions development is accelerated while in high activity conditions development is decelerated thus reducing the variability in the density versus LogE curve (the characteristic curve) caused by changes in development time.

## Patentansprüche

1. Verfahren zur Entwicklung eines bildweise exponierten Silberhalogenid-Farbmaterials unter Erzielung sensitometrischer Ergebnisse von verminderter Variabilität, das umfaßt
die Durchführung der Farbentwicklung in einer wäßrigen Farbentwicklerlösung, die eine Farbentwicklerverbindung enthält, in Gegenwart von einer oder einer Kombination von Pyrazolidinon-Silberhalogenidentwicklerverbindugen der allgemeinen Formel: worin R¹ und R² jeweils für Wasserstoff stehen oder eine Alkoxygruppe mit 1 bis 4 Kohlenstoffatomen und worin R³ und R⁴ jeweils Wasserstoffatome sind oder eine Alkylgruppe mit 1 bis 10 Kohlenstoffatomen,
wobei gilt, daß einer der Reste R¹ oder R² eine Alkoxygruppe ist oder einer der Reste R³ oder R⁴ eine Alkylgruppe mit 3 bis 7 Kohlenstoffatomen,
eingearbeitet in das Silberhalogenid-Farbmaterial in einer inaktiven Form, aus der die aktive Form in der alkalischen Entwicklerlösung freigesetzt wird, wobei die Natur des oder der Pyrazolidinon-Silberhalogenidentwicklerverbindungen derart ist, daß unter Bedingungen geringer Aktivität die Entwicklung beschleunigt wird, während unter Bedingungen hoher Aktivität die Entwicklung verzögert wird, unter Verminderung der Variabilität in der Dichte in Abhängigkeit von der LogE-Kurve (der Charakteristikkurve), verursacht durch Veränderungen in der Entwisklungsdauer.

2. Verfahren nach Anspruch 1, bei dem das Pyrazolidinon-Entwicklungsmittel ebenfalls in der Farbentwicklerlösung enthalten ist.

3. Verfahren nach Anspruch 1 oder 2, bei dem mindestens einer der Reste R¹ und/oder R² eine Alkoxygruppe mit 1 bis 4 Kohlenstoffatomen ist, R³ für ein Wasserstoffatom oder eine Alkylgruppe mit 1 bis 4 Kohlenstoffatomen steht und R⁴ ein Wasserstoffatom ist oder eine Hydroxyalkylgruppe mit 1 bis 4 Kohlenstoffatomen.

4. Verfahren nach Ansprüchen 1 oder 2, bei dem R¹, R² und R³ jeweils für Wasserstoffatome stehen und R⁴ eine Alkylgruppe mit 3 bis 7 Atomen ist.

5. Verfahren nach einem der Ansprüche 1 bis 4, bei dem das Pyrazolidinon-Entwicklungsmittel 1-(4-Methoxyphenyl)-3-pyrazolidon; 1-(3,4-Dimethoxyphenyl)-3-pyrazolidon oder 1-Phenyl-4-n-pentylpyrazolidon ist.

6. Verfahren nach einem der Ansprüche 2 bis 5, bei dem das Pyrazolidinon-Entwicklungsmittel in der Entwicklerlösung in einer Konzentration von 0,05 bis 0,5 g/l vorliegt.

7. Verwendung von einem oder von mehreren Pyrazolidonen zur Verminderung der sensitometrischen Variabilität von entwickelten photographischen Silberhalogenid-Farbmaterialien, wobei die Pyrazolidinone die allgemeine Formel (I) haben: worin R¹ und R² jeweils für ein Wasserstoffatom oder eine Alkoxygruppe mit 1 bis 4 Kohlenstoffatomen stehen und R³ und R⁴ jeweils stehen für ein Wasserstoffatom oder eine Alkylgruppe mit 1 bis 10 Kohlenstoffatomen,
wobei gilt, daß einer der Reste R¹ oder R² für eine Alkoxygruppe steht oder einer der Reste R³ oder R⁴ für eine Alkylgruppe mit 3 bis 7 Kohlenstoffatomen,
und wobei das oder die Pyrazolidinone während der Farbentwicklung vorliegen, die durchgeführt wird in einer wäßrigen Farbentwicklerlösung, und wobei das oder die Pyrazolidinone derart sind, daß unter Bedingungen geringer Aktivität die Entwicklung beschleunigt wird, wohingegen unter Bedingungen hoher Aktivität die Entwicklung verzögert wird, unter Verminderung der Variabilität der Dichte in Abhängigkeit von der LogE-Kurve (der Charakteristikkurve), verursacht durch Veränderungen in der Entwicklungsdauer.

## Revendications

1. Procédé de développement d'un matériau en couleurs aux halogénures d'argent exposé suivant une image pour donner des résultats sensitométriques de variabilité réduite qui comprend
la mise en oeuvre du développement chromogène dans une solution aqueuse de développement chromogène contenant un agent développateur chromogène en présence d'un ou d'une combinaison d'agents développateurs des halogénures d'argent du type pyrazolidinone de formule générale : dans laquelle
R¹ et R² sont chacun l'hydrogène ou un groupe alcoxy en C₁-C₄ et
R³ et R⁴ sont chacun l'hydrogène ou un groupe alkyle en C₁-C₁₀,
pourvu que l'un ou l'autre de R¹ et R² soit un groupe alcoxy ou que l'un ou l'autre de R³ et R⁴ soit un groupe alkyle en C₃-C₇,
incorporé dans ledit matériau en couleurs aux halogénures d'argent sous une forme inactive à partir de laquelle la forme active est libérée dans la solution révélatrice alcaline, la nature du ou des agents développateurs des halogénures d'argent du type pyrazolidinone étant telle que, dans des conditions de faible activité, le développement est accéléré, tandis que, dans des conditions d'activité élevée, le développement est ralenti, réduisant ainsi la variabilité de la courbe de densité en fonction de logE (courbe caractéristique) provoquée par des variations de la durée de développement.

2. Procédé selon la revendication 1, dans lequel l'agent développateur du type pyrazolidinone est également contenu dans la solution de révélateur chromogène.

3. Procédé selon la revendication 1 ou 2, dans lequel l'un au moins de R¹ et/ou R² est un groupe alcoxy en C₁-C₄, R³ est l'hydrogène ou un groupe alkyle en C₁-C₄ et R⁴ est l'hydrogène ou un groupe hydroxyalkyle en C₁-C₄.

4. Procédé selon la revendication 1 ou 2, dans lequel R¹, R² et R³ sont des atomes d'hydrogène et R⁴ est un groupe alkyle en C₃-C₇.

5. Procédé selon l'une quelconque des revendications 1 à 4, dans lequel l'agent développateur du type pyrazolidinone est la 1-(4-méthoxyphényl)-3-pyrazolidone, la 1-(3,4-diméthoxyphényl)-3-pyrazolidone ou la 1-phényl-4-n-pentylpyrazolidone.

6. Procédé selon l'une quelconque des revendications 2 à 5, dans lequel l'agent développateur du type pyrazolidinone est présent dans la solution de révélateur à une concentration de 0,05 à 0,5 g/l.

7. Utilisation d'une ou plusieurs pyrazolidinones pour réduire la variabilité sensitométrique des matériaux photographiques en couleurs aux halogénures d'argent traités, dans laquelle les pyrazolidinones répondent à la formule générale (I) : dans laquelle
R¹ et R² sont chacun l'hydrogène ou un groupe alcoxy en C₁-C₄ et
R³ et R⁴ sont chacun l'hydrogène ou un groupe alkyle en C₁-C₁₀,
pourvu que l'un ou l'autre de R¹ et R² soit un groupe alcoxy ou l'un ou l'autre de R³ et R⁴ soit un groupe alkyle en C₃-C₇,
et dans laquelle la ou les pyrazolidinones sont présentes pendant le développement chromogène mis en oeuvre dans une solution aqueuse de développement chromogène et sont telles que, dans des conditions de faible activité, le développement est accéléré, tandis que, dans des conditions d'activité élevée, le développement est ralenti, réduisant ainsi la variabilité de la courbe de densité en fonction de logE (courbe caractéristique) provoquée par des variations de la durée de développement.
